

**1**

2,892,793

**LUBRICANT COMPOSITION**

William T. Stewart, El Cerrito, Donovan R. Wilgus, Berkeley, and Frank A. Stuart, Orinda, Calif., assignors to California Research Corporation, San Francisco, Calif., a corporation of Delaware

No Drawing. Application September 19, 1957  
Serial No. 684,834

13 Claims. (Cl. 252—56)

This invention relates to a novel lubricant composition. More particularly, the invention is directed to a novel lubricant composition which is unusually effective in the lubrication of internal combustion engines.

Improvements in the design of internal combustion engines during recent years and changes in the conditions of modern-day engine operation have emphasized the need for more effective lubricant composition. The lubricant compositions must enable the engines to operate for prolonged periods at the highest possible efficiency under widely varying conditions. To do this, they must reduce friction, thereby increasing the efficiency of the engines, and at the same time decrease attrition of certain rubbing parts, such as piston rings and cylinder walls.

In the operation of internal combustion engines, substantial amounts of solid deposits tend to occur on the interior surfaces. These deposits have a serious effect on the operating efficiency of the engines, since they add greatly to the friction of rubbing surfaces and interfere with proper circulation of the lubricants. For the same reason, the wear of the rubbing surfaces is greatly accelerated, resulting eventually in a serious loss of power, and more frequent replacement or overhaul of the piston rings and cylinder walls becomes necessary. Lubricant compositions which prevent or minimize the formation of solid deposits within the internal combustion engines are therefore highly desirable.

The operation of internal combustion engines is also affected by the corrosive attack on metal surfaces of moisture and acids formed in the combustion of the fuels. This leads to additional wear of piston rings and cylinder walls, as well as other metal surfaces. The ability of lubricant compositions to decrease wear due to corrosion in internal combustion engines is thus an important attribute.

The formation of solid deposits within internal combustion engines and the wear of rubbing surfaces is considerably aggravated by the conditions under which such engines are commonly used in this day. In the stopping and starting of automobile engines during city driving, for example, the engines are repeatedly started in cold condition and operated for short periods of time, insufficient for them to reach the more efficient higher temperatures. Increased amounts of partial oxidation products of the fuels, and also of the lubricant compositions to a somewhat less degree, are thus formed and never fully exhausted from the engine. These products are generally either insoluble or sparingly soluble in lubricating oils. Even the slightly soluble ones tend to polymerize or conglomerate, with the formation of insoluble masses which deposit out on contact with engines surfaces. Other oxidation products of the fuel and lubricant composition

**2**

are acidic by nature and combine with moisture under the relatively cold operation conditions of city driving to cause further undesirable wear of the piston rings and cylinder walls.

5 Lubricant compositions have been prepared with additives to inhibit the formation of solid deposits and reduce the wear of rubbing parts. Detergents have been added to prevent or minimize engine deposits. These detergents are generally metal-containing compounds such as calcium petroleum sulfonate, calcium cetyl phosphate, calcium phenyl stearate and the like. Metal salts of petroleum sulfonic acids and other metallo-organic compounds, particularly those having a basic reaction, have been added to counteract the effect of moisture and acidic products on metal surfaces within the engines.

Lubricant compositions with additives of the above type have not been completely satisfactory in the lubrication of modern internal combustion engines under present-day operating conditions. Their ability to solubilize oxidation products and avoid the formation of solid deposits has been somewhat limited at the lower temperatures and the corrosion of metal surfaces has not been satisfactorily inhibited. A further disadvantage of the metal-containing additives employed heretofore 20 has been that they may form an ash upon combustion which deposits out upon surfaces within the internal combustion engine, thereby resulting in a decrease of engine efficiency and an increase in wear of engine parts, as described above.

30 In the present invention, a new and unusually effective lubricant composition has been discovered comprising a major portion of an oil of lubricating viscosity and a minor portion, sufficient to enhance the detergent characteristics of the composition, of an oil-soluble mixture 35 of (A) the copolymer of at least one monomer selected from the group consisting of (1) a fatty acid ester of an unsaturated alcohol, said fatty acid containing up to 30 carbon atoms and said unsaturated alcohol being selected from the group consisting of  $\alpha$  and  $\beta$ -unsaturated alcohols 40 containing up to 20 carbon atoms, (2) 1-olefins of 2 to 30 carbon atoms, and (3) vinyl and allylalkyl ethers having 1 to 30 carbon atoms in the alkyl group with a monomer of the group consisting of maleic anhydride and alkyl, cycloalkyl, aryl, alkaryl and aralkyl  $\alpha, \alpha'$ -substituted maleic anhydrides containing up to 20 carbon atoms, said monomers being in approximately 1:1 molar ratio, and (B) a copolymer comprising as its monomers 45 a member of the group consisting of maleic anhydride and alkyl, cycloalkyl, aryl, alkaryl and aralkyl  $\alpha, \alpha'$ -substituted maleic anhydrides containing up to 20 carbon atoms and at least one olefinically unsaturated oil solubilizing monomer having an aliphatic hydrocarbon group of 4 to 30 carbon atoms, at least one of said (A) and (B) copolymers being partially esterified with a member 50 of the group consisting of polyalkylene glycols and ethers thereof in which the alkylene groups contain from 2 to 7 carbon atoms each and the alkyl groups contain from 1 to 30 carbon atoms each and said (A) and (B) copolymers being in the weight ratio of 0.15 to 5 parts of (A) for each part of (B), and a portion of the maleic anhydride and substituted maleic anhydride in the copolymers being present as a derivative thereof selected from the group consisting of a free carboxylic acid, an amide, N-alkyl amides and amine salts, alkyl esters, and N-alkyl amides and amine salts and alkyl esters having at least 55 one hydrogen of their alkyl group, but not more than one- 60 65

half thereof, substituted by a polar group. Copolymers containing the amides, amine salts and esters are a distinct species from those having the free carboxylic acid group and copolymeric mixtures containing them possess highly useful detergent characteristics in lubricant compositions which could not be predicted from the unmixed copolymers alone.

Novel lubricant compositions of the type according to the present invention as described above are outstanding in the lubrication of internal combustion engines, even under the more stringent operating conditions commonly encountered in the engines of today. Remarkably little or no deposits are formed on the interior surfaces of internal combustion engines employing these compositions thus providing more efficient operation while at the same time decreasing undesirable wear of rubbing surfaces within the engine. Wear of engine parts due to corrosive attack is also effectively inhibited by the use of the compositions of the invention. Such benefits are all the more noteworthy, since they are apparently attained without any loss of additive or other detrimental effect on the lubricant composition. This is wholly unlike previous experiences with conventional compositions for such purposes where the additive is used up due to its combination with the objectionable deposit-forming and wear-inducing partial oxidation by-products of lubricating oil bases and fuels. A still further important advantage of the lubricant compositions lies in the fact that the detergent and wear-inhibiting additive does not contain metal which could itself contribute to the formation of deposits upon combustion.

The fatty acid ester of an unsaturated alcohol in component (A) of the mixture of copolymers, as already mentioned, may contain up to 30 carbon atoms in both the fatty acid and the unsaturated alcohol, and the unsaturated alcohol may be either an  $\alpha$  or  $\beta$ -unsaturated alcohol. Illustrative fatty acid esters of this type are:

|                        |                         |
|------------------------|-------------------------|
| Vinyl formate          | Methylallyl palmitate   |
| Vinyl palmitate        | Crotyl acetate          |
| Vinyl caprylate        | Crotyl stearate         |
| Vinyl eicosanoate      | 1-propenyl isobutyrate  |
| Allyl acetate          | 1-hexenyl acetate       |
| Allyl laurate          | 2-decetyl caproate      |
| Allyl stearate         | 2-decetyl laurate       |
| Allyl 2-ethylhexanoate | 1-hexadecenyl myristate |
| Methylallyl caproate   | 2-eicosenyl palmitate   |

Preferred esters are those in which the unsaturated alcohol is a  $\beta$ -unsaturated alcohol of from 3 to 7 carbon atoms and the fatty acid contains from 8 to 20 carbon atoms. Esters of this type, such as allyl palmitate, allyl stearate, methylallyl eicosanoate and 2-hexenyl laurate, particularly the allyl esters of the higher fatty acids, give the most effective detergents and wear inhibitors when incorporated in the copolymers of the lubricant compositions in accordance with this invention.

In the present description, the terms "higher fatty acids" and "higher alkyl esters" are employed in their commonly accepted sense and refer to fatty acids containing at least 8 carbon atoms and alkyl esters in which the alkyl group contains at least 8 carbon atoms. Ordinarily, not more than 30 carbon atoms are necessary in such groups for the purposes of this invention.

For present purposes the fatty acid esters of unsaturated alcohols are preferred in the (A) component for their effectiveness in the oil-soluble mixtures of copolymers according to the invention.

A distinct species of the invention within the terms of the general statement above may also be obtained by including in copolymer (B) a fatty acid ester of an unsaturated alcohol of the type described in connection with copolymer (A). Copolymers of this specific type have been found to produce lubricant compositions having superior detergency under certain conditions compared to compositions in which the fatty acid ester of unsaturated alcohol was omitted from the (B) copolymer.

On the other hand, lubricant compositions containing copolymeric mixtures wherein the (B) component is the copolymer of the maleic anhydride compound and the olefinically unsaturated oil solubilizing monomer alone without the unsaturated alcohol ester constitute a very effective species of the invention having excellent detergent properties which would not be expected from the performance of the unmixed copolymers.

Described in another way, the (B) component of the copolymer mixtures employed in the lubricant compositions of the invention may include other monomers of the type described herein, along with the maleic anhydride or substituted maleic anhydride and oil solubilizing monomer. The two species of invention mentioned in the preceding paragraph are particular types of lubricant compositions containing mixed copolymers in which the (B) component is a copolymer of monomers selected from at least the first two classes of the group consisting of (1) maleic anhydride and alkyl, cycloalkyl, aryl, alkyl aryl and aralkyl  $\alpha, \alpha'$ -substituted maleic anhydrides containing up to 20 carbon atoms, (2) an olefinically unsaturated oil solubilizing monomer having an aliphatic hydrocarbon group of 4 to 30 carbon atoms and (3) a fatty acid ester of an unsaturated alcohol in which the fatty acid contains up to 30 carbon atoms and the unsaturated alcohol is a member of the group consisting of  $\alpha$  and  $\beta$ -unsaturated alcohols containing up to 20 carbon atoms.

The 1-olefins of 2 to 30 carbon atoms are well known and readily available from a number of sources including the polymerization of olefins such as ethylene and propylene, cracking of hydrocarbons, dehydrogenation of hydrocarbons, dehydration of alcohols and the like. They are essentially aliphatic in structure and contain a single olefinic double bond in the 1-position. Preferred 1-olefins are those containing 6 to 24 carbon atoms. The following are illustrative:

|                  |                      |
|------------------|----------------------|
| Ethylene         | Hexene-1             |
| 2-ethylhexene-1  | Octadecene-1         |
| Diisobutylene    | Eicosene-1           |
| Triisobutylene   | 4-octylcyclohexene-1 |
| Propylene trimer | 3-phenylhexadecene-1 |
| Dodecene-1       | p-Octylstyrene       |
| Hexadecene-1     | Vinylcyclohexane     |

45 The vinyl and allyl alkyl ethers, as already mentioned, have 1 to 30 carbon atoms in the alkyl group. Preferred are those containing 4 to 22 carbon atoms in the alkyl portion thereof. Illustrative ethers include:

|                                         |                                       |
|-----------------------------------------|---------------------------------------|
| Vinyl methyl ether                      | Allyl methyl ether                    |
| Vinyl ethyl ether                       | Methylallyl octadecyl ether           |
| Vinyl n-butyl ether                     | Propenyl 2-ethylhexyl ether           |
| Vinyl 2-ethylhexyl ether                | Crotyl n-octyl ether                  |
| Allyl n-butyl ether                     | Isopropenyl dodecyl ether             |
| Allyl isobutyl ether                    | 1-decetyl butyl ether                 |
| Allyl cyclohexyl ether                  | 1-eicosenyl decyl ether               |
| Allyl 4,4,8,8-tetramethylidocosyl ether | Vinyl p-octylphenyl ether             |
| Methylallyl n-hexyl ether               | Methylallyl p-tert. butylphenyl ether |
| Methylallyl n-decyl ether               | 1-decetyl p-cetylphenyl ether         |
| Methylallyl 2-ethylhexyl ether          | 1-decetyl 2-phenylbutyl ether         |
| Methylallyl propyl ether                |                                       |

50 60 The maleic anhydride and  $\alpha, \alpha'$ -substituted maleic anhydrides containing up to 20 carbon atoms in component (A) of the copolymer may be illustrated by the following structural formula:



more than 16 carbon atoms. Illustrative anhydrides of this type are maleic anhydride, citraconic anhydride, otherwise described as  $\alpha$ -methyl maleic anhydride,  $\alpha$ -hexyl maleic anhydride,  $\alpha, \alpha'$ -diethyl maleic anhydride,  $\alpha$ -methyl  $\alpha'$ -cyclohexyl maleic anhydride,  $\alpha, \alpha'$ -diphenyl maleic anhydride,  $\alpha$ -methyl  $\alpha'$ -benzyl maleic anhydride,  $\alpha$ -tertiary butylphenyl maleic anhydride,  $\alpha, \alpha'$ -dixyl anhydride and  $\alpha$ -cetyl maleic anhydride. Maleic anhydride is presently preferred, since it is most readily available and provides block copolymers of the greatest effectiveness in the lubricant compositions according to this invention.

In component (B) of the copolymers, the maleic anhydride and  $\alpha, \alpha'$ -substituted maleic anhydrides containing up to 20 carbon atoms may be the same as in the (A) component described in the preceding paragraph, or they may be different, so long as they fall within the terms of the general description set out above.

The olefinically unsaturated oil solubilizing compound containing an aliphatic hydrocarbon group of from 4 to 30 carbon atoms may be selected from a wide variety of well-known oil solubilizing monomers which have been employed heretofore in the production of polymers for addition to lubricant compositions to modify their physical properties, that is, their viscosity indexes and pour point characteristics. The aliphatic hydrocarbon group and the polymerizable olefinic double bond are the two essential features of these oil solubilizing compounds. The aliphatic group is branched or straight chain alkyl or cycloalkyl in structure. This is illustrated by radicals such as butyl, isobutyl, 2-ethylhexyl, cyclohexyl, tetradeethyl, stearyl, eicosenyl, oleyl and ricinoleyl. The aliphatic hydrocarbon groups are linked to the polymerizable olefinic double bonds or vinylene groups either directly or by an oxygen-containing group, as in the case of ethers, esters, ketones.

The olefinically unsaturated oil solubilizing monomers of component (B) may also be illustrated by the following general formula:



in which  $R_1$  and  $R_2$  are members of the group consisting of hydrogen and hydrocarbyl radicals of from 4 to 30 carbon atoms, at least one of which contains an aliphatic hydrocarbon group of from 4 to 30 carbon atoms as described above,  $G$  and  $G'$  are members of the class consisting of oxy ( $-\text{O}-$ ), carbonyl



and carboxyloxy



groups and combinations thereof with not more than two alkylene groups of from 1 to 7 carbon atoms each and  $n$  and  $n'$  are 0 or 1. When  $R_1$  and  $R_2$  are hydrocarbyl radicals, they may be alkyl, cycloalkyl, alkenyl, cycloalkenyl, aryl, alkaryl or aralkyl in structure as illustrated by radicals such as 2-ethylhexyl, cyclohexyl, hexenyl, cyclohexenyl, phenyl, naphthyl, tertiary butylphenyl, benzyl, etc.

The olefinically unsaturated oil solubilizing compound referred to above may also be an  $\alpha$  or  $\beta$ -unsaturated alcohol ester of a fatty acid, either like or unlike the ester monomer already described in connection with copolymer (A) and copolymer (B). Mixtures of the oil solubilizing monomers may be employed if desired.

The following olefins, ethers and esters are offered as illustrations of suitable oil-soluble monomers for prepara-

tion of the (B) copolymers employed in the lubricant compositions of the invention:

#### OLEFINS

|   |                        |                        |
|---|------------------------|------------------------|
| 5 | Hexene-1               | Octadecene-1           |
|   | 2-ethylhexene-1        | Eicosene-1             |
|   | Di- and triisobutylene | 4-octylcyclohexene-1   |
|   | Propylene trimer       | 3-phenylhexadecene-1   |
|   | Dodecene-1             | p-Octylstyrene         |
|   | Hexadecene-1           | Vinylcyclohexane       |
|   | Cyclohexene            | p-Tertiarybutylstyrene |

10

|    |                                        |                                     |
|----|----------------------------------------|-------------------------------------|
| 10 | Vinyl n-butyl ether                    | Methallyl octadecyl ether           |
|    | Vinyl 2-ethylhexyl ether               | Propenyl 2-ethylhexyl ether         |
|    | Allyl n-butyl ether                    | Crotyl n-octyl ether                |
|    | Allyl isobutyl ether                   | Isopropenyl dodecyl ether           |
|    | Allyl cyclohexyl ether                 | 1-decenyl butyl ether               |
|    | Allyl 4,4,8,8-tetramethyldocosyl ether | 1-eicosenyl decyl ether             |
| 15 | Methallyl n-hexyl ether                | Vinyl p-octylphenyl ether           |
|    | Methallyl n-decyl ether                | Methallyl p-tert. butylphenyl ether |
|    | Methallyl 2-ethylhexyl ether           | 1-decetyl p-cetylphenyl ether       |
|    |                                        | 1-decetyl 2-phenylbutyl ether       |

#### ETHERS

|    |                                        |                                       |
|----|----------------------------------------|---------------------------------------|
| 20 | Cyclohexyl methacrylate                | Cyclohexyl 2-dodecenoate              |
|    | Decyl vinylacetate                     | Isooctyl $\alpha$ -chloroacrylate     |
|    | P-isobamylphenyl 2-hexadecenoate       | 4-p-tolylbutyl 2-octadecenoate        |
|    | Undecyl cinnamate                      | Methylcyclohexyl 2-ethyl-2-hexenoate  |
|    | 5-ethylidocosyl crotonate              | Octadecyl isocrotonate                |
|    | N-butyl 2-eicosenote                   | p-Tert. amylophenyl octadecyl maleate |
|    | p-Hexadecylphenyl 2-ethylhexyl maleate | o-Tolyl 2-octadecylcyclohexyl maleate |
| 25 | Dihexadecyl maleate                    | o-Nonylphenyl-hexadecyl maleate       |
|    | Mono-2-ethylhexyl maleate              | Di-methylcyclohexyl maleate           |
|    | Di-dodecyl maleate                     | Di-2-ethylhexyl fumarate              |
|    | Di-dodecyl citraconate                 | Di-dodecyl mesaconate                 |
|    | Monohexadecyl itaconate                | o-Tolyl octadecyl itaconate           |
|    | 1-decetyl laurate                      | Isopropenyl palmitoleate              |
|    | Dodecyl acrylate                       | 1-hexadecenyl myristate               |
| 30 | Isobutyl $\alpha$ -decylacrylate       | Hexadecyl methacrylate                |
|    | Dimonophenoxyethyl methacrylate        | Cetylphenoxyethyl methacrylate        |

#### KETONES

|    |                                         |                            |
|----|-----------------------------------------|----------------------------|
| 35 | Vinyl n-butyl ketone                    | Methallyl octadecyl ketone |
|    | Vinyl 2-ethylhexyl ketone               | 1-decetyl butyl ketone     |
|    | Allyl cyclohexyl ketone                 | 1-eicosenyl decyl ketone   |
|    | Allyl 4,4,8,8-tetramethyldocosyl ketone | Vinyl p-octylphenyl ketone |

Although any of the olefinically unsaturated oil solubilizing compounds described above will give effective copolymer compositions for lubricant compositions in accordance with the present invention, higher alkyl esters of  $\alpha, \beta$ -unsaturated monocarboxylic acids of from 3 to 8 carbon atoms are preferred. Representative acids of this type are the acrylic, methacrylic, crotonic, tiglic, angelic,  $\alpha$ -ethylacrylic,  $\alpha$ -methylcrotonic,  $\alpha$ -ethylcrotonic,  $\beta$ -ethylcrotonic,  $\alpha$ -butylcrotonic, hydroisorbic,  $\alpha$ -ethylhydroisorbic and  $\alpha$ -propylhydroisorbic acids and the like. Even more desirable are the alkyl esters of acrylic and methacrylic acids containing from 10 to 20 carbon atoms in the alkyl groups, since they are found to provide highly superior polymers for the lubricant compositions of the invention and are obtainable in commercial quantities.

The polyalkylene glycols and alkyl ethers thereof used in the esterification of the copolymeric (A) and (B) components of the copolymer additives for the lubricant compositions of the invention contain from 2 to 7 carbon atoms in each alkylene group and 1 to 30 carbon atoms in each alkyl group, as already mentioned. Poly-1,2-alkylene glycols and their alkyl ethers having molecular weights between 106 and 10,000 are preferred. Such glycols may be obtained by polymerizing 1,2-alkylene oxides or mixtures thereof in the presence of a catalyst and a suitable initiator for the reaction such as water, monohydric alcohol, in the case of the alkyl ethers, mercaptan and the like. The preparation of polyglycol compounds of this type has been fully described heretofore in U.S. Patents 2,448,664, 2,457,139, for example, and therefore, requires no detailed discussion here.

For present purposes, the most suitable poly-1,2-alkylene glycols are those derived from ethylene oxide or from 1,2-propylene oxide or mixtures thereof and their alkyl ethers of 1 to 18 carbon atoms per alkyl group which have molecular weights or average molecular weights between about 200 and 2000. Copolymers partially esterified with these polyalkylene glycols are found to pro-

vide the most effective detergent and wear inhibiting compositions.

The following polyalkylene glycols containing from 2 to 7 carbon atoms each are illustrative of the types described above.



Polyethylene glycol mixtures having average molecular weights of 200, 400, 1000, 1540 or 2000.

Poly-1,2-propylene glycol mixtures having average molecular weights of 425 or 1025.

The copolymers of the lubricant compositions of the invention, as mentioned in the general statement given above, have a portion of the maleic anhydride and substituted maleic anhydride monomer present as a derivative thereof selected from the group consisting of a free carboxylic acid, an amide, N-alkyl amides and amine salts, alkyl esters and n-alkyl amides and amine salts and alkyl esters having at least one hydrogen of their alkyl group but not more than one-half thereof substituted by a polar group. Such maleic anhydride and substituted maleic anhydride type compounds in the copolymers may be represented by the following formula:



in which  $M_1$  and  $M_2$  represent the balance of the copolymer, the  $R$ 's are hydrogen or hydrocarbyl radicals of the type already discussed,  $R_1$  and  $R_2$ , which may be the same or different, are groups selected from the class consisting of polyoxyalkyleneoxy groups obtained when polyalkylene glycols of the above-described types are reacted with maleic anhydride, an hydroxyl group, an amide group,  $N$ -alkyl amide and amine salt groups, alkoxy groups and  $N$ -alkyl amide and amine salt groups and alkoxy groups having at least one hydrogen of their alkyl group, but not more than one-half thereof, substituted by a polar group.

In the case of the N-alkyl amide and amine salt groups, as well as the N-alkyl amide and amine salt groups having alkyl group hydrogens substituted by polar groups,  $R_1$  and  $R_2$  have the structure:



in which formulae the  $R_3$ 's are hydrogen atoms or alkyl 75

and polar substituted alkyl groups, and the  $R_4$ 's are alkyl or polar substituted alkyl groups similar to the  $R_3$  groups. Preferred alkyl groups are the lower alkyl groups, that is, those containing from 1 to 7 carbon atoms. The polar groups may be any of the class of groups which are known to impart polarity to an organic molecule. Illustrative groups of this type are the amino, bromo, carboxy, chloro, cyano, imido, imino, isocyanato, mercapto, nitramino, nitro, nitroso, sulfo and thiocyanato groups. Preferred polar groups are the amido, amino, hydroxy and mercapto groups.

In the case of the alkoxy and polar substituted alkoxy groups, the alkyl groups and polar substituted alkyl groups may be as described above in connection with the 15) amine salt and amide groups.

Illustrative N-polar substituted alkyl amide and amine salt groups of the preceding types are as follows:

|    |                                                                                                                                                                                                                                    |
|----|------------------------------------------------------------------------------------------------------------------------------------------------------------------------------------------------------------------------------------|
| 20 | Ethanolamine salt<br>Diethanolamine salt<br>Mercaptoethylamine salt<br>Diethylenetriamine salt<br>Tetraethylenepentamine salt                                                                                                      |
| 25 | Dihydroxyethyl ethylenediamine salt<br>Triethanolamine salt<br>2,5-dimethylpiperazine salt<br>3-hydroxymorpholine salt<br>N-(2-hydroxyethyl)-amide                                                                                 |
| 30 | N-(2-mercaptoproethyl)-amide<br>N-(2-aminoethyl)-amide<br>N-(4-aminobutyl)-amide<br>N-(4-aminohexyl)-amide<br>N-(3-azapentyl)-amide                                                                                                |
| 35 | N-(2-nitrohexyl)-amide<br>N-(2,3-dihydroxypropyl)-amide<br>N-(2-hydroxy-5-mercaptopentyl)-amide<br>N-(4-hydroxycyclohexyl)-amide<br>N-(2-ethyl-6-aminohexyl)-amide                                                                 |
| 40 | 3-nitromorpholine amide<br>N-ethyl-N-(2-hydroxyethyl)-amide<br>N,N-di(2-hydroxyethyl)-amide<br>N-(2-hydroxyethyl)-N-aminomethyl-<br>N-(2-nitroethyl)-amide                                                                         |
| 45 | N-(2-hydroxy-6-phenylhexyl)-amide<br>N-(2-hydroxyethyl)-N-(3-aza-5-hydroxy-<br>The amide of 2-hydroxyethyl p-aminobenzoic acid<br>The amide of pentaerythritol mono-p-aminobenzoate<br>The amide of 2-hydroxyethyl 3-aminobutyrate |

Alcohols which provide substituted alkyl ester groups, or the alkyl portion of the polar substituted alkoxy groups as they are termed above, include:

|                               |                                   |
|-------------------------------|-----------------------------------|
| 2-hydroxyethyl alcohol        | Inositol                          |
| 2-aminoethyl alcohol          | 2,2,6,6-tetramethylolcyclohexanol |
| 2-hydroxypropyl alcohol       | 3-aza-5-aminopentyl alcohol       |
| 3-hydroxypropyl alcohol       | N-(2-aminoethyl)-3-aza-5-hydroxy  |
| 2,3-dihydroxypropyl alcohol   | pentyl alcohol                    |
| 3-oxa-5-hydroxypropyl alcohol | 3-aza-5-hydroxypentyl alcohol     |
| Erythritol                    | Sucrose                           |
| Pentaerythritol               | 2-mercaptopethyl alcohol          |
| Cyclohexyl pentaerythritol    | 3-mercaptopropyl alcohol          |
| Dipentaerythritol             | 2-nitroethyl alcohol              |
| Tri pentaerythritol           | 3,6-dihydroxycyclohexyl alcohol   |
| Sorbitol                      | 2-aza-propyl alcohol              |
| 65 Mannitol                   | 3,5-dihydroxyphenyl alcohol       |
| Arabitol                      | 2,2-dimethylbutyl alcohol         |
|                               | 3,5-dinitrocyclohexyl alcohol     |

It will be noted from the above examples that the polar substituted alkyl groups are straight chain alkyl, branched alkyl or cycloalkyl in structure and contain at least one polar group. In the case of the polar substituted alkyl ester groups, or alkoxy groups as they have also been termed, it is desirable that at least half, and not less than 75% of the carbon atoms in the alkyl portion be attached

to the polar groups. As already mentioned, preferred alkyl groups are the lower alkyl groups of from 1 to 7 carbon atoms. Although the amido, amino, hydroxyl and mercapto groups constitute a preferred class of polar groups, the greatest preference is given to the amino and hydroxyl groups, particularly the latter.

In the preparation of the copolymer additives for lubricant compositions according to this invention the ratio of the various monomeric and polymeric components to one another is such that the final mixture of copolymers is soluble in the mineral oil or other oil of lubricating viscosity in amounts sufficient to enhance the detergent characteristics and wear inhibiting properties of the composition. Generally, the ratios are such that the lubricant compositions contain at least 0.1% by weight and preferably 1% or more of the copolymer mixture on the basis of the entire lubricant composition. Inasmuch as the various monomeric components described hereinbefore possess differing oil solubilizing effects, it is convenient to test the oil solubility of the copolymers until the proper ratios are determined.

It has been found that copolymers having the desired degree of oil solubility as described above and possessing detergent enhancing and wear inhibiting properties generally contain monomeric ratios which fall within certain numerical ranges. In the copolymeric (B) component of the mixture containing an unsaturated alcohol ester as previously described, from about 0.25 to 4 moles of the  $\alpha$  or  $\beta$ -unsaturated alcohol ester of a fatty acid is present for each mole of the maleic anhydride compounds. The olefinically unsaturated oil solubilizing monomer in the copolymeric (B) component is ordinarily present in molar proportions 5 to 50 times that of the combined amount of  $\alpha$  or  $\beta$ -unsaturated alcohol fatty acid ester and maleic anhydride compound. Stated otherwise, this usually amounts to from about 83 to 98 mole percent of the (B) component. Ordinarily from about 0.15 to about 5 parts by weight of copolymeric component (A) are present for each part by weight of the copolymeric (B) component in the mixture of copolymers. Preferably, the weight ratio of (A) to (B) is in the range of from 0.25 to 2 of (A) for each part of (B). The polyalkylene glycol esterifying the copolymeric (A) and (B) components is such that a total of from about 2 to 75% of the maleic acid anhydride of the (A) and (B) components is esterified. This means that usually from about 0.04 to 1.5 mole of polyalkylene glycol is present for each mole of maleic anhydride or that from about 1 to 25 weight percent of the final polymer mixture is polyalkylene glycol present as an ester group. As will be apparent from the last-mentioned properties, the copolymers of the compositions according to the invention are characterized by the presence of free acid or carboxyl groups which are in turn suitably converted to amide, amine salt or ester derivatives thereof, since only one-half of a maleic acid anhydride group is often esterified.

As already mentioned, the maleic anhydride compound and the other monomer of the (A) component are present in approximately 1:1 molar ratio. Minor variations of, for example, one-half a mole either way are permissible to provide a molar ratio of the two monomers in the range of from 0.5:1.5 to 1.5:0.5.

The copolymer additives of the lubricant compositions of the invention have apparent molecular weights as determined by standard light scattering methods of at least 2,000 and preferably at least about 8,000. For practical purposes, molecular weights of from 100,000 to 1 million are most suitable from the standpoint of viscosity and other physical characteristics of the polymeric additives.

Several methods of preparing the copolymers for the lubricant compositions of the invention may be employed. Monomers containing reaction groups may be first poly-

merized and then the desired hydrocarbyl substituents added by reaction with the group. This is illustrated in situations where acrylic acid or methacrylic acid monomers are polymerized and the polymeric product then esterified with a higher alkyl alcohol.

In the preparation of the copolymeric components or polymeric intermediates therefor, conventional bulk, solution or emulsion methods may be employed. Polymerization initiators such as benzoyl peroxide, acetyl peroxide, tertiary butyl hydroperoxide or an azo initiator such as  $\alpha, \alpha'$ -azodiisobuteronitrile are usually employed in amounts of 0.1 to 10%. Inert solvents may be used as needed to facilitate handling of the materials and to maintain the reaction mixture in a homogeneous condition. The copolymerization reactions are ordinarily carried out at temperatures of about 170 to 300° F., depending on the nature of the solvent, the concentration of the reactants, the catalyst and reaction times.

After the copolymeric (A) and (B) components have been prepared, they may be esterified separately with the desired polyalkylene glycol or its monoether or the two copolymers may be mixed and esterified together with the polyalkylene glycol or ether reactant which reacts with a portion of the maleic anhydride groups in both copolymers. This esterification is preferably carried out in the presence of catalysts such as p-toluene sulfonic acid monohydrate. Solvents such as toluene, xylene and the like are used to facilitate the reaction, and the temperatures vary from about 200 to 400° F. in accordance with known esterification procedures.

Any of the well-known types of oils of lubricating viscosity are suitable base oils for the compositions of the invention. They include hydrocarbon or mineral lubricating oils of naphthenic, paraffinic, and mixed naphthenic and paraffinic types. They may be refined by any of the conventional methods such as solvent refining and acid refining. Synthetic hydrocarbon oils of the alkylene polymer type or those derived from coal and shale may also be employed. Alkylene oxide polymers and their derivatives such as the propylene oxide polymers and their ethyl esters and acetyl derivatives in which the terminal hydroxyl groups have been modified are also suitable. Synthetic oils of the dicarboxylic acid ester type including dibutyl adipate, di-2-ethylhexyl sebacate, di-n-hexyl fumaric polymer, dilauryl azelate, and the like may be used. Alkyl benzene types of synthetic oils such as tetradecyl benzene, etc., are also included. Liquid esters of acids of phosphorus including tricresyl phosphate, diethyl esters of decane phosphonic acid, and the like may also be employed. Also suitable are the polysiloxane oils of the type of polyalkyl-, polyaryl-, polyalkoxy- and polyaryloxy siloxanes such as polymethyl siloxane, polymethylphenyl siloxane, and polymethoxyphenoxy siloxane and silicate ester oils such as tetraalkyl- and tetraaryl silicates of the tetra-2-ethylhexyl silicate and tetra-p-tert.-butylphenyl silicate types.

As further illustrations of the invention according to the above description, the following examples are offered showing the preparation of the novel copolymeric detergents and wear inhibitors and lubricant compositions containing them. Unless otherwise specified, the proportions are given on a weight basis.

#### Example I

To a glass reaction flask equipped with stirring means, thermometer, reflux condenser and dropping funnel were charged 98 grams (1 mole) of maleic anhydride and 324 grams (1 mole) of allyl stearate along with about 10 cc. of benzene. The contents of the flask were heated to about 225° F. while stirring. About 6.3 grams of benzoyl peroxide dissolved in 100 cc. of benzene was added to the mixture over a period of about 4 hours. The temperature was maintained between about 200 and 230° F. by heating or cooling as necessary during the addi-

tion. 4.2 grams of tertiary butyl hydroperoxide was then added, following which the mixture was thoroughly stirred and allowed to stand for 18 hours at 218° F. The mixture thus obtained was distilled to a temperature of 370° F. under a vacuum equal to about 1 mm. of mercury pressure. The product was a glassy appearing copolymer containing equimolar proportions of maleic anhydride and allyl stearate and having an apparent molecular weight of about 90,000 as determined by standard light scattering methods.

254 grams (1 mole) of lauryl methacrylate and 5 grams (0.05 mole) of maleic anhydride were added to a glass reaction flask equipped with mechanical stirrer, reflux condenser and thermometer. The mixture was heated to about 200° F. for a period of about 2 hours, during which time 2 grams of tertiary butyl peroxide was added. The temperature was maintained at 215-225° F. during the addition by either heating or cooling as required. When the addition of the catalyst was completed, the mixture was allowed to stand for about 18 hours at 215-225° F. The reaction mixture was then stripped by distillation at 380° F. at 1 mm. mercury pressure to give a viscous oil soluble polymer shown by analysis to have a molal ratio of lauryl methacrylate to maleic anhydride of approximately 20/1.

120 grams of the lauryl methacrylate-maleic anhydride (20/1) copolymer and 80 grams of the allyl stearate-maleic anhydride (1/1) copolymer were mixed with 16.8 grams of polyethylene glycol monomethyl ether having an average molecular weight of about 550, 0.34 gram of p-toluene sulfonic acid monohydrate catalyst and sufficient xylene to permit refluxing slowly at 300° F. in a glass reaction flask of the above type. The mixture was refluxed for about nine hours while stirring. Another 33.6 grams of the polypropylene glycol monomethyl ether and 0.6 gram of p-toluene sulfonic acid catalyst were then added. Xylene was permitted to distill off until the temperature reached 350° F. at which temperature the reaction was maintained for about five hours. The mixture was stripped to a temperature of 370° F. at a pressure of 1 mm. of mercury. An amber colored, viscous material soluble in oil was thus obtained which consisted of the mixture of (A) allyl stearate-maleic anhydride (1/1) copolymer and (B) lauryl methacrylate-maleic anhydride (20/1) copolymer partially esterified with polyethylene glycol monomethyl ether having a molecular weight of about 550.

#### Example II

An allyl stearate-maleic anhydride (1/1) copolymer having an apparent molecular weight of about 90,000 was prepared as described above. To a glass reaction flask equipped with stirrer, and reflux thermometer were charged 380 grams of lauryl methacrylate (1.5 mole) and 5 grams of maleic anhydride (0.05 mole). The mixture was heated to about 200° F. and 2 grams of tertiary butyl peroxide and 2 grams of benzoyl peroxide were added over a period of about 2 hours. The mixture was heated or cooled as necessary during the addition to maintain the temperature at 215-225° F. Following the addition, the mixture was heated for about 18 hours at 215-225° F. It was then stripped to a temperature of 380° F. at 1 mm. mercury pressure to yield a lauryl methacrylate-maleic anhydride (30/1) copolymer in the form of an amber colored, viscous material having an apparent molecular weight of about 500,000.

120 grams of the lauryl methacrylate-maleic anhydride copolymer and 80 grams of the allyl stearate-maleic anhydride copolymer obtained in the above preparations were mixed in a glass reaction vessel with 15.0 grams of polyethylene glycol having an average molecular weight of about 300, 0.3 gram of p-toluene sulfonic acid catalyst and enough xylene to permit slow refluxing at about 300° F. While stirring, the mixture was refluxed for about 9 hours at 300° F. Then an additional 25.0 grams of

5 polyethylene glycol and 0.68 gram of the p-toluene sulfonic acid catalyst were added. The xylene was stripped off until the temperature reached 350° F. at which point it was held for about 5 hours. The remaining solvent 10 was then removed by distillation up to 370° F. at 1 mm. mercury pressure. The product was a mixture of (A) allyl stearate-maleic anhydride (1/1) copolymer and (B) lauryl methacrylate-maleic anhydride (30/1) copolymer partially esterified with polyethylene glycol having an average molecular weight of about 400. It was a highly viscous, amber colored material which was soluble in oil.

#### Example III

The 1/1 copolymer of allyl stearate and maleic anhydride was prepared by the procedure of the above examples.

15 Into a glass reaction flask was placed a mixture of 127 grams of lauryl methacrylate (0.5 mole) and 5 grams of maleic anhydride (0.05 mole). The ingredients were 20 mixed and heated to about 220° F. 2 grams of tertiary butyl hydroperoxide and 2 grams of benzoyl peroxide were then added slowly over a period of about 2 hours. The reaction flask was heated or cooled as necessary to maintain the temperature at 215-225° F. during this period. After the mixture had been heated for an additional 18 hours at about 220° F., it was stripped to 380° F. at 1 mm. mercury pressure. The lauryl methacrylate-maleic anhydride (10/1) copolymer thus obtained was a viscous, amber colored oil soluble material.

25 80 grams of the allyl stearate-maleic anhydride copolymer and 120 grams of the maleic anhydride-lauryl methacrylate copolymer prepared above were mixed in the glass reaction flask and reacted with 16.8 grams of polyethylene glycol monomethylether having an average molecular weight of about 550. The catalyst was 0.34 gram of p-toluene sulfonic acid and the reaction conditions and purification steps were the same as outlined in the above examples. The final product was a copolymeric mixture of (A) maleic anhydride-allyl stearate 1/1 copolymer and (B) maleic anhydride-lauryl methacrylate 1/10 copolymer partially esterified with the polyethylene glycol monomethylether. It was viscous and amber colored in appearance and was soluble in oil.

#### Example IV

324 grams (1 mole) of allyl stearate, 98 grams (1 mole) of maleic anhydride and 10 cc. of benzene were charged to a three-necked flask fitted with a stirrer, thermometer, reflux condenser and dropping funnel. The mixture was heated to 220-225° F. with stirring. A solution of 6.3 grams of benzoyl peroxide in 100 cc. of benzene was then added over a period of 3 to 4 hours during which time the temperature was maintained between 200 and 230° F. by heating or cooling as required. After 55 about 15 to 20 cc. of the catalyst and benzene solution had been added, polymerization began and toluene was added slowly as required to facilitate stirring of the mixture. Following the addition of all of the benzoyl peroxide and benzene solution, 4.2 grams of tertiary butyl hydroperoxide was added. The mixture was thoroughly stirred and then let stand for about 18 hours at 218° F.

60 The product obtained above was stripped to 370° F. at 1 mm. mercury pressure to give 415 grams of a mixture comprising unreacted allyl stearate and maleic anhydride and a glassy appearing copolymer containing equimolar quantities of allyl stearate and maleic anhydride. It had an apparent molecular weight of about 90,000 as determined by standard light scattering methods.

To 211 grams of the stripped allyl stearate-maleic anhydride copolymeric mixture was added 317 grams of lauryl methacrylate. The combined materials were then heated, with stirring to 260-270° F. until homogeneous. The solution was then cooled to 220-225° F. and a mixture of 0.7 gram of benzoyl peroxide and 0.7 gram of 75 tertiary butyl hydroperoxide was added over a period of

1 to 2 hours while maintaining the temperature between 220-230° F. After about 3 hours' reaction time, 1.4 grams more of each of the above catalysts was added. The mixture was stirred and then allowed to stand for about 18 hours at 218° F.

The mixture obtained above was stripped to 370° F. at 1 mm. pressure to remove unreacted lauryl methacrylate. The resulting product was a viscous oil-soluble mixture shown by analyses to comprise (A) allyl stearate-maleic anhydride 1/1 copolymer and (B) allyl stearate-maleic anhydride-lauryl methacrylate copolymer with a molal ratio of 1/1/15.

To 200 grams of the mixture of copolymers obtained above were added 16.8 grams of polyethylene glycol monomethyl ether having an approximate molecular weight of about 550, 0.34 gram of p-toluene sulfonic acid monohydrate catalyst and sufficient xylene to give slow refluxing at 300° F. This mixture was refluxed at 300° F. with stirring for about 9 hours. At this point, an additional 39.0 grams of the polyethylene glycol monomethyl ether and 0.68 gram of p-toluene sulfonic acid monohydrate catalyst were then added. Xylene was withdrawn until the temperature rose to 350° F. The reaction mixture was held at this temperature for about 5 hours, following which the xylene was stripped off by distillation up to 370° F. under a vacuum equal to 1 mm. mercury pressure.

The mixture of copolymers of (A) allyl stearate-maleic anhydride 1/1 copolymer and (B) allyl stearate-maleic anhydride-lauryl methacrylate 1/1/15 copolymer each esterified with polyethylene glycol monomethyl ether having an average molecular weight of 550 as obtained in the above experiment was a viscous, oil-soluble, amber colored material. It contains about 10% free unreacted polyethylene glycol monomethyl ether and may be used as is in oils of lubricating viscosity to impart enhanced detergency and wear-inhibiting properties, or it may be further purified by dissolving in 4 volumes of benzene and precipitating the polymers with 20 to 25 volumes of methanol.

#### Example V

In this example a maleic anhydride-allyl stearate copolymer was prepared by the method described in Example IV above. It had an apparent molecular weight of about 90,000 as determined by standard light scattering methods.

A maleic anhydride-lauryl methacrylate-allyl stearate copolymer was synthesized by mixing 254 grams (1 mole) of lauryl methacrylate, 5 grams (0.05 mole) of maleic anhydride and 16.2 grams (0.05 mole) of allyl stearate in a three-necked reaction flask fitted with a stirrer, condenser and thermometer in accordance with the procedure of Example IV. The mixture was heated to 220° F. and 2 grams of benzoyl peroxide was added over a period of 2 hours. During this time, the temperature was maintained at 215-225° F. by either heating or cooling as required. Following the addition of the catalyst, the mixture was held at 215-225° F. for about 18 hours and then stripped to 380° F. at 1 mm. mercury pressure to yield 260 grams of a viscous, oil-soluble polymer shown by analysis to contain lauryl methacrylate, allyl stearate and maleic anhydride in a molal ratio of approximately 20/1/1.

A mixture of 80 grams of the allyl stearate-maleic anhydride copolymer and 120 grams of the lauryl methacrylate-allyl stearate-maleic anhydride copolymer prepared above was combined with 16.8 grams of a polyethylene glycol monomethyl ether having an average molecular weight of approximately 550, 0.34 gram of p-toluene sulfonic acid monohydrate catalyst and sufficient xylene to permit refluxing slowly at 300° F. in the reaction flask described previously. The contents of the flask were refluxed for about 9 hours at 300° F. while stirring. At this point, 39.0 grams of the polyethylene glycol mono-

ethyl ether were added along with 0.68 gram of catalyst. Xylene was boiled off until the temperature reached 350° F. and the reaction mixture then maintained under these conditions for about 5 hours. Following this, xylene was stripped off by distillation at 370° F. under a vacuum equal to a pressure of about 1 mm. of mercury. The product thus obtained was an amber colored viscous material which was soluble in oil.

10

*Example VI*

A copolymer of allyl stearate and maleic anhydride containing equimolar proportions of the components was prepared in the manner outlined in Examples IV and V. It had an apparent molecular weight of about 90,000 as determined by standard light scattering methods.

15

381 grams of lauryl methacrylate (1.5 moles), 5 grams of maleic anhydride (0.05 mole) and 16.2 grams of allyl stearate (0.05 mole) were mixed in a three-necked flask fitted with mechanical stirrer, a reflux condenser and thermometer. The mixture was then heated to about 200° F., following which 3 grams of tertiary butyl hydroperoxide and 3 grams of benzoyl peroxide were added during a period of 2 hours, the temperature being maintained at 215-225° F. by heating or cooling as required. The mixture was heated at 215-225° F. for another 18 hours and then stripped by distillation to a temperature of 380° F. at 1 mm. mercury pressure. Approximately 370 grams of maleic anhydride-lauryl methacrylate-allyl stearate copolymer was obtained. The molal ratio of lauryl methacrylate, allyl stearate and maleic anhydride in this copolymer was approximately 30/1/1.

20

80 grams of the allyl stearate maleic anhydride copolymer and 120 grams of the maleic anhydride-lauryl methacrylate-allyl stearate copolymer prepared above were mixed with 16.8 grams of polyethylene glycol having an average molecular weight of about 400 in the reaction vessel described above. 0.34 gram of p-toluene sulfonic acid monohydrate catalyst and sufficient xylene to give slow refluxing at about 300° F. were added. The mixture was refluxed at about 300° F. for about 9 hours with stirring. An additional 39.0 grams of the polyethylene glycol and 0.68 grams of the p-toluene sulfonic acid catalyst were then added, and xylene was allowed to distill off until the temperature reached 350° F. The reaction mixture was held at this temperature for about 5 hours, following which the xylene was stripped off by distilling up to 370° F. at 1 mm. mercury pressure.

25

The product obtained above was a highly viscous, oil-soluble, amber colored polymer. It was further purified by dissolving it in 4 volumes of benzene and then precipitating it from the benzene with 20-25 volumes of methanol. The precipitated polymer was then freed of solvent by distilling up to 370° F. at 1 mm. mercury pressure to give the purified mixture of the partial polyethylene glycol esters of the copolymers of maleic anhydride-allyl stearate, 1/1 copolymer and lauryl methacrylate-allyl stearate-maleic anhydride 30/1/1 copolymer.

30

*Example VII*

A mixture containing a copolymer of maleic anhydride and allyl stearate in equimolar proportions was prepared in this example by the procedure as outlined in Example IV above. As previously, the apparent molecular weight was approximately 90,000. A copolymer of allyl stearate, maleic anhydride and lauryl methacrylate was then prepared by the reaction of lauryl methacrylate with the mixture containing the maleic anhydride-allyl stearate 1/1 copolymer. This product, as in the case of Example IV, was shown by analysis to be a mixture of 2 copolymers, (A) the allyl stearate-maleic anhydride 1/1 copolymer and (B) allyl stearate-maleic anhydride-lauryl methacrylate 1/1/15 copolymer.

35

125 grams of the mixture of copolymers obtained above

was combined with 40.0 grams of polyethylene glycol monolauryl ether. 0.60 gram of p-toluene sulfonic acid catalyst was then added. Xylene was distilled off until the temperature rose to about 350° F. The reaction mixture was then held at this temperature for about 5 hours, following which the xylene was stripped by permitting it to distill off until a temperature of 370° F. at 1 mm. mercury pressure was reached.

The product obtained above was purified by dissolving it in 4 volumes of benzene and precipitating the polymer with 20-25 volumes of methanol. The precipitated polymer was then freed of solvents by distillation up to 370° F. under a vacuum equal to a pressure of 1 mm. of mercury. This polymer was an amber colored, viscous, oil-soluble material which was shown by analysis to be the mixture of copolymers of (A) allyl stearate-maleic anhydride 1/1 copolymer and (B) allyl stearate-maleic anhydride-lauryl methacrylate 1/1/15 copolymer each partially esterified with the lauryl ether of polyethylene glycol having a molecular weight of about 550.

#### Example VIII

In this example a copolymer of allyl stearate and maleic anhydride having a 1/1 molal ratio and an apparent molecular weight of about 90,000 was prepared as described in the above examples. 211 grams of the unpurified reaction mixture containing this copolymer was then reacted with 507 grams of inhibitor-free lauryl methacrylate in the same manner as previously described in connection with Examples IV and VII to give a mixture of 2 copolymers, (A) the allyl stearate-maleic anhydride 1/1 copolymer and (B) the allyl stearate-maleic anhydride-lauryl methacrylate copolymer with a molal ratio of 1/1/24.

100 grams of the mixture of copolymers obtained above was mixed with 54 grams of polyethylene glycol monomethyl ether having an average molecular weight of approximately 550, and 0.5 gram of p-toluene sulfonic acid monohydrate catalyst was added. The reaction mixture was heated at 320° F. for about two hours and then at 350° F. for about 14 hours, following the same procedure as given in the above examples.

The final product obtained above was stripped by vacuum distillation, extracted with hot methanol, and then stripped again. It was a viscous, amber colored, polymeric material consisting of a mixture of copolymers of (A) maleic anhydride-allyl stearate 1/1 copolymer and (B) maleic anhydride-allyl stearate-lauryl methacrylate copolymer having a 1/1/24 molal ratio, each esterified with a polyethylene glycol monomethyl ether having an average molecular weight of approximately 550.

#### Example IX

An allyl stearate-maleic anhydride 1/1 copolymer was prepared in this example by the same procedure as outlined in the preceding examples.

127 grams of lauryl methacrylate (0.5 mole), 5 grams of maleic anhydride (0.05 mole) and 16.2 grams of allyl stearate (0.05 mole) were mixed together and heated to about 220° F. A mixture of 2 grams of tertiary butyl hydroperoxide and 2 grams of benzoyl peroxide was added slowly over a period of about 2 hours, during which time the temperature was maintained at 215-225° F. by heating or cooling as it became necessary. Following this addition, the mixture was heated at about 220° F. for about 18 hours and then stripped to 380° F. at 1 mm. of mercury pressure to yield a viscous, amber colored, oil-soluble polymer containing lauryl methacrylate, maleic anhydride and allyl stearate in a molal ratio of approximately 10/1/1.

A mixture of 80 grams of the allyl stearate-maleic anhydride 1/1 copolymer and 120 grams of the maleic anhydride-allyl stearate-lauryl methacrylate 1/1/10 copolymer prepared above was reacted with 16.8 grams of

polyethylene glycol monoethyl ether having an average molecular weight of about 550 in the presence of 0.34 gram of p-toluene sulfonic acid monohydrate catalyst. Following this, another 34.8 grams of polyethylene glycol was added. The reaction conditions and purification steps were the same as outlined in Example IV. The final product was a viscous, amber colored material consisting of a mixture of esterified copolymers of (A) maleic anhydride-allyl stearate 1/1 copolymer and (B) maleic anhydride-allyl stearate-lauryl methacrylate 1/1/10 copolymer each esterified with polyethylene glycol monoethyl ether.

#### Example X

100 grams of allyl stearate and maleic anhydride copolymer in 1/1 molal ratio prepared as described above, 150 grams pearl oil, 21 grams polyethylene glycol 550 molecular weight monomethyl ether, 0.43 gram p-toluene sulfonic acid catalyst and 420 cc. xylene were mixed and heated at reflux temperature (300° F.) for 9 hours. 50 grams more polyethylene glycol 550 molecular weight monomethyl ether and 0.86 gram catalyst were added and xylene withdrawn to raise reflux temperature to 350° F. The mixture was maintained at this temperature for 5 hours.

The above product was purified by chromatography on silica gel. Solvents were first removed by vacuum distillation and the crude product dissolved in 2½ liters of cyclohexane. This solution was passed through a column of silica gel which was then washed with 2 liters of fresh cyclohexane. The cyclohexane solutions after passing through the column, were combined and stripped to yield 120 grams of purified partial polyglycol esters of the allyl stearate and maleic anhydride copolymer.

Maleic anhydride, lauryl methacrylate and allyl stearate copolymer was prepared as in Example V. 100 grams of this polymer was esterified as above using the same quantities, times and temperatures.

After esterification, solvents were removed by vacuum distillation and 142 grams of the crude product was dissolved in 4.4 liters of benzene-cyclohexane mixture of 15:85 ratio. This solution was passed through a column of silica gel which was washed with 7 liters of the same solvent mixture. 76 grams of the pure partial polyglycol ester was recovered by distillation of these solvents. The ratio of (A) component/(B) component/polyglycol was 36/54/12.

#### Example XI

252 grams of octadecene-1 (1 mole) and 98 grams maleic anhydride (1 mole) were mixed and warmed to 215° F. with stirring. A solution of 7 grams of benzoyl peroxide in 116 cc. benzene was added over a period of 2 hours. During this time thickening occurred but the mixture remained stirrable. At this time 5 cc. of tertiary butyl hydroperoxide was added and the mixture let stand at 212° F. for a further 18 hours.

Crude product was stripped to 350° F. at one millimeter to yield approximately at 1:1 copolymer of octadecene-1 and maleic anhydride.

100 grams of this product were mixed with 181 grams of maleic anhydride, lauryl methacrylate and allyl stearate copolymer, prepared as in Example II. 24 grams of polyethylene glycol 550 molecular weight monomethyl ether, 0.48 gram p-toluene sulfonic acid catalyst and enough xylene such that reflux occurred at 300° F. Mixture was refluxed at 300° F. with stirring for 9 hours, at which time a further 55 grams of polyethylene glycol 550 molecular weight monomethyl ether and 0.95 gram of p-toluene sulfonic acid catalyst were added and xylene removed to raise reflux temperature to 350° F. Heating and stirring were continued at this temperature for 5 hours. The crude product was stripped of solvents, 297 grams of this crude product were dissolved in xylene (1 liter) and passed through a silica gel column. The column was washed with 1 liter of fresh xylene and the

xylene solutions combined and stripped to yield a mixture of the partial polyglycol esters of octadecene-1 and maleic anhydride copolymer and maleic anhydride, lauryl methacrylate and allyl stearate copolymer. The ratio of octadecene-1 and maleic anhydride copolymer/maleic anhydride, lauryl methacrylate and allyl stearate copolymer/polyglycol was 36/55/15.

*Example XII*

98 grams (1 mole) of maleic anhydride and 156 grams (1 mole) of vinyl 2-ethylhexyl ether and 900 cc. benzene were mixed and warmed to reflux. 8 grams benzoyl peroxide in a solution of 50 cc. benzene were added over 10 minutes. The mixture was refluxed with stirring for 4 hours. The polymer was precipitated from benzene with hexane and dried to yield 219 grams of an essentially 1/1 copolymer.

75 grams of the above copolymer and 187 grams of maleic anhydride, lauryl methacrylate and allyl stearate copolymer (prepared as in Example V), 22 grams polyethylene glycol 550 molecular weight monomethyl ether, and 0.45 gram p-toluene sulfonic acid were mixed with sufficient xylene to cause refluxing at 300° F., at which temperature the mixture was stirred for 9 hours. An additional 52 grams polyethylene glycol 550 molecular weight monomethyl ether and 19 grams catalyst were added and xylene removed to raise reflux temperature to 350° F. Stirring at this temperature continued for 5 hours.

203 grams of the crude stripped product were dissolved in a 1:1 mix of benzene and xylene (2 liters) and purified by treatment with silica gel as in Example XI to yield 156 grams of the partial polyglycol ester of the mixture of 1:1 maleic anhydride and vinyl 2-ethylhexyl ether copolymer and the 1/20/1 maleic anhydride, lauryl methacrylate and allyl stearate copolymer. The ratio of maleic anhydride and vinyl 2-ethylhexyl ether copolymer/maleic anhydride, lauryl methacrylate and allyl stearate copolymer/polyethylene glycol 550 molecular weight monomethyl ether was 32/55/10.

*Example XIII*

147 grams maleic anhydride (1½ moles), 176 grams vinyl 2-ethylhexyl ether (1.13 moles), and 122 grams allyl stearate (0.38 mole) were mixed and heated to 210° F. 9 grams benzoyl peroxide in 90 cc. benzene were added over 3½ hours and held at 217° F. for a further 18 hours. Crude product was stripped to 380° F. at 0.5 millimeter to yield 415 grams of a 1/75/25 copolymer of maleic anhydride, vinyl-2-ethylhexyl ether, allyl stearate.

75 grams of this copolymer and 160 grams maleic anhydride, lauryl methacrylate and allyl stearate copolymer (prepared as in Example V) were esterified and purified by the same methods used in Example XII to yield a mixture of the partial polyethylene glycol 550 molecular weight monomethyl-ether esters of the two copolymers. The ratio of maleic anhydride, vinyl-2-ethylhexyl ether and allyl stearate copolymer/maleic anhydride, lauryl methacrylate and allyl stearate copolymer/polyethylene glycol 550 molecular weight monomethyl ether was 34/55/15.

*Example XIV*

Following the procedure of the above examples, a copolymer of methallyl stearate and maleic anhydride was prepared using equimolar proportions. One part of the copolymer thus obtained was mixed with 1.5 parts of maleic anhydride, lauryl methacrylate and allyl stearate copolymer in 1/20/1 mole ratio prepared as in Example V. The mixture was then esterified with polyethylene glycol 550 molecular weight monomethyl ether to give partial ester in which the ratio of methallyl stearate and maleic anhydride copolymer/maleic anhydride, lauryl

methacrylate and allyl stearate copolymer/polyethylene glycol 550 molecular weight monomethyl ether was 37/55/10.

*Example XV*

5 In the same manner as described above, a 1:1 copolymer of vinyl stearate and maleic anhydride was prepared and mixed with one and one-half times its weight of maleic anhydride, lauryl methacrylate and allyl stearate copolymer in 1/20/1 mole ratio. The mixture was esterified with polyethylene glycol 550 molecular weight monomethyl ether to give a partial ester in which the ratio of vinyl stearate and maleic anhydride copolymer/maleic anhydride, lauryl methacrylate and allyl stearate copolymer/polyethylene glycol 550 molecular weight monomethyl ether was 35/55/12.

In accordance with the present invention, very superior lubricant compositions are obtained when mixed copolymeric additives of the type described above are added 10 to a base oil of lubricating viscosity. The additives may be employed in any amount sufficient to enhance the detergency and wear inhibiting properties of the compositions. Excellent detergency and wear inhibiting properties are imparted to lubricating oils by the addition of 15 from about 0.1 to 10% by weight based on the composition of the copolymers. The present invention finds its preferred embodiment in lubricant compositions containing the copolymer mixture in amounts of from about 20 1 to 5%, since such proportions are sufficient to give 25 detergency and wear protection over prolonged periods of time when the compositions of this invention are employed in an engine, as distinguished from compositions previously employed in the prior art for similar purposes. Another unusual feature of the lubricant compositions of the invention is the fact that the polymers 30 are sufficiently soluble in oil to permit the production of lubricating oil concentrates containing proportions of additive mixture as high as 75% by weight based on the composition of the concentrate. Such concentrates are 35 exceptionally suitable for diluting with lubricating base oils in the preparation of final lubricant compositions.

The effectiveness of the mixed polymers of the invention as detergents and wear inhibitors is evaluated in a series of engine tests. The method employed in these

45 tests is that described for the "FL-2 Engine Test" in the June 21, 1948, Report of the Co-ordinating Research Council.

In accordance with this method, the compounded oil is employed as the crankcase lubricant in a 6-cylinder Chevrolet engine operated with a low grade 50 gasoline especially prone to cause engine deposits. A jacket temperature of 95° F. and a crankcase oil temperature of 155° F. are maintained. The engine is operated at 2500 r.p.m. under a load of 45 brake horsepower for 40 hours.

"Cold" engine conditions normally experienced 55 in city driving are thus closely simulated. At the end of each test the engine is dismantled and the amount of engine deposits on the piston determined and expressed as the Average Piston Varnish Rating. This value is obtained by visually rating the amount of deposit on each piston and averaging the individual ratings

60 so obtained for the various pistons on a scale of 0 to 10 with 10 representing the absence of any deposits.

The piston ring wear encountered with the various 65 lubricant compositions employed in these tests is also illustrative of the effectiveness of the compositions. This wear, measured in terms of milligrams per hour, is considered to be satisfactory if it does not exceed 4 milligrams per hour.

The lubricant compositions in the tests contain a solvent 70 refined SAE-30 mineral lubricating oil as a base oil with additives as indicated in the following table of test results. Other oils of lubricating viscosity are similarly benefited when compounded with additives to produce lubricant compositions according to the present invention.

TABLE I

| (A) Component                                                                  | (B) Component                                                                         | Polyalkylene glycol                                            | Proportions of (A),<br>(B) and polyalkylene<br>glycol | Percent<br>by weight<br>additive<br>in com-<br>position | Average<br>piston<br>varnish<br>rating | Piston<br>ring<br>wear,<br>mg./hr. |
|--------------------------------------------------------------------------------|---------------------------------------------------------------------------------------|----------------------------------------------------------------|-------------------------------------------------------|---------------------------------------------------------|----------------------------------------|------------------------------------|
| None (base oil alone)                                                          | None (base oil alone)                                                                 | None (base oil alone)                                          | None (base oil alone)                                 | 0                                                       | 3.5                                    | 5.0                                |
| Allyl stearatemaleic anhydride, 1/1 copolymer.                                 | Lauryl methacrylate-maleic anhydride, 20/1 copolymer.                                 | Polyethylene glycol, 550 mole weight monomethyl ether.         | 35/54/11                                              | 2.5                                                     | 8.5                                    | 2.8                                |
| Do.                                                                            | Lauryl methacrylate-maleic anhydride, 30/1 copolymer.                                 | Polyethylene glycol, 400 mole weight.                          | 37/56/7                                               | 2.5                                                     | 7.8                                    | 3.2                                |
| Do.                                                                            | Lauryl methacrylate-maleic anhydride, 10/1 copolymer.                                 | Polyethylene glycol, 550 mole weight monomethyl ether.         | 38/57/5                                               | 2.5                                                     | 6.0                                    | 3.7                                |
| None                                                                           | Lauryl methacrylate-maleic anhydride, 20/1 copolymer.                                 | do                                                             | 95.8/4.2                                              | 2.5                                                     | 5.0                                    | 3.7                                |
| Allyl stearatemaleic anhydride, 1/1 copolymer.                                 | None                                                                                  | do                                                             | 80/20                                                 | 2.5                                                     | 4.1                                    | 4.0                                |
| Do.                                                                            | Allyl stearatemaleic anhydride-lauryl methacrylate, 1/1/15 copolymer.                 | do                                                             | 36/55/9                                               | 2.5                                                     | 9.7                                    | 2.7                                |
| Do.                                                                            | Allyl stearatemaleic anhydride-lauryl methacrylate, 1/1/20 copolymer.                 | do                                                             | 36/55/9                                               | 1.5                                                     | 8.6                                    | 3.1                                |
| Do.                                                                            | Allyl stearatemaleic anhydride-lauryl methacrylate, 1/1/30 copolymer.                 | do                                                             | 37/56/7                                               | 2.5                                                     | 9.5                                    | 2.9                                |
| Do.                                                                            | Allyl stearatemaleic anhydride lauryl methacrylate, 1/1/15 copolymer.                 | Polyethylene glycol, 400 mole weight.                          | 38.6/57.9/3.5                                         | 2.5                                                     | 8.5                                    | 3.2                                |
| Do.                                                                            | Allyl stearatemaleic anhydride lauryl methacrylate, 1/1/10 copolymer.                 | Polyethylene glycol, 550 mole weight monolauryl dialkyl ether. | 34/51.5/14.5                                          | 2.5                                                     | 9.2                                    | 2.9                                |
| Do.                                                                            | Allyl stearatemaleic anhydride lauryl methacrylate, 1/1/10 copolymer.                 | Polyethylene glycol, 550 mole weight monomethyl ether.         | 38.5/57.5/4                                           | 1.5                                                     | 6.5                                    | 3.6                                |
| Do.                                                                            | do                                                                                    | do                                                             | 37.8/56.7/5.5                                         | 2.5                                                     | 7.8                                    | 3.5                                |
| Do.                                                                            | None                                                                                  | Polyglycol, 550 mole weight monomethyl ether.                  | 88.5/11.5                                             | 2.5                                                     | 4.5                                    | 3.9                                |
| None                                                                           | Allyl stearatemaleic anhydride-lauryl methacrylate, 1/1/20 copolymer.                 | do                                                             | 91/9                                                  | 2.5                                                     | 5.5                                    | 3.5                                |
| Vinyl stearatemaleic anhydride, 1/1 copolymer.                                 | do                                                                                    | do                                                             | 38/58/4                                               | 2.5                                                     | 7.2                                    | 3.7                                |
| Allyl stearatemaleic anhydride, 1/1 copolymer.                                 | Allyl stearatemaleic anhydride-vinyl-2-ethyl-hexoate, 1/1/20 copolymer.               | Polyethylene glycol, 550 mole weight monomethyl ether.         | 30/60/10                                              | 2.5                                                     | 7.7                                    | 3.6                                |
| Octadecene-1-maleic anhydride, 1/1 copolymer.                                  | Maleic anhydride, lauryl methacrylate and allyl stearate copolymer, 20/1/1 copolymer. | do                                                             | 34/55/15                                              | 1.5                                                     | 7.2                                    | -----                              |
| Vinyl 2-ethylhexyl ether-maleic anhydride, 1/1 copolymer.                      | do                                                                                    | do                                                             | 32/55/10                                              | 1.5                                                     | 7.1                                    | -----                              |
| Vinyl 2-ethylhexyl etherallyl stearatemaleic anhydride, 0.75/0.25/1 copolymer. | do                                                                                    | do                                                             | 34/55/15                                              | 1.5                                                     | 7.1                                    | -----                              |

As shown by the illustrative test data of the above table, the lubricant compositions of the invention are outstanding detergents and wear inhibitors under the most severe conditions encountered in the low temperature operation of internal combustion engines. The base oil alone gives an average piston varnish rating and piston ring wear of 3.5 and 5.0, respectively, whereas the improved compositions of the invention containing the illustrative polymeric additives give results in the order of 9.7 and 2.7, respectively. Excellent results of 8.5 varnish and 2.8 wear are also obtained in mixtures where the unsaturated alcohol ester is omitted from the (B) component.

It may also be seen from the above test results that the unusual effectiveness of the lubricant compositions of the invention is entirely unexpected and unpredictable. Although the polyethylene glycol esters of the allyl stearate-maleic anhydride (A) component and the allyl stearate-maleic anhydride-lauryl methacrylate or lauryl methacrylate-maleic anhydride (B) component are fairly effective when employed separately in the lubricant compositions, compared to the base oil alone, they are only about one-half as effective as the copolymer mixture containing lubricant compositions in accordance with the present invention.

In addition to the foregoing illustrations of the polymeric compositions according to the invention, the following examples are submitted to show the methods of preparing mixed copolymers containing polar groups other than the free carboxylic acid groups referred to

above. The first of these methods deals with the preparation of polar group-containing, mixed copolymers of the type listed in Examples XVI, XXV and XXII to XXXV, inclusive of the following table. The (A) and (B) copolymers and polyalkylene glycol are combined in the manner already described in the previous examples. The introduction of the polar group-containing component, hereinafter referred to as component (C), is then accomplished by subjecting the glycol esterified (A) and (B) copolymers to the usual reactions. For example, amide and alkoxy derivatives are prepared by reacting the mixed copolymers of (A) and (B) esterified by polyglycol with the amine or alcohol having the desired characteristics which will produce the corresponding amide or alkoxy group. The reaction is carried out in a suitable solvent such as xylene at temperatures in the range from 270 to 400° F. using an acid catalyst such as p-toluenesulfonic acid. Because of the relatively low rate of reaction usually encountered with these products, a 25 to 100% excess of the amine or alcohol is employed and the unreacted portion is removed by distillation where the reactant is volatile or by precipitation of the product from the hydrocarbon solvent with a polymeric anti-solvent. Where poly-functional amines or alcohols such as ethylenediamine or ethylene glycol are employed for the (C) component, a relatively dilute reaction medium is favored (30 to 80% solvent) to control cross-linking reactions which, if permitted to occur to any appreciable extent, may produce hydrocarbon-insoluble, gel-like polymers. Thio esters and substituted thio esters are pro-

duced in a similar manner. Ammonium salts are prepared simply by adding the amine to a solution of the glycol-esterified mixed copolymers and warming at 200 to 300° F. for a short period until the reaction is complete. In other preparations, particularly where a mono-functional polar-type substituent is employed, the (C) component is substituted on the mixture of (A) and (B) copolymers or on the (A) or (B) copolymer alone prior to reaction of the (A) and (B) mixture with the polyalkylene glycol.

In the second series of preparations, Examples XXVI to XXXI, inclusive, the method of preparing mixed copolymers containing polar group constituents follows a different route. In this type of synthesis the polar group component (C) is added to copolymer (A) and/or (B) during its preparation. Since the maleic anhydride content of copolymer (A) is ordinarily much higher than that of copolymer (B), as already mentioned, it is generally preferred to make the substitution of the polar group component (C) in copolymer (A). In a preparation of this type, the copolymer (A) or (B) is prepared

by the usual methods already described in connection with the preceding examples. A portion of the maleic anhydride, however, is replaced by a suitable derivative of the anhydride such as the imide, the half-amide, the diamide, alkyl amides, thio esters, esters, ammonium salts and the like. The resulting copolymer of (A) and/or (B) thus includes the (C) component. The preparation of the final product, the mixed copolymers, is then accomplished by completing the reaction of (A) and/or (B) and (C) copolymers with the remaining unused copolymers, that is, (A) or (B) and the polyalkylene glycol or ether thereof.

The choice between the above two methods for the preparation of mixed copolymers in accordance with the present invention is generally controlled by ease of synthesis of the maleic acid anhydride derivative and its polymerization rate, or the ease with which it copolymerizes with the other monomers involved.

The above methods will yield novel products, as illustrated by the following examples, which will impart the indicated properties to lubricant compositions.

TABLE II

| Example No. | (A) Component                                                                           | (B) Component                                                           | Polyalkylene glycol                                         | Maleic anhydride polar substituent group (C)                   | Proportions of (A), (B) poly-alkylene glycol and (C) | Percent by weight additive in composition | Average piston varnish rate | Piston ring wear, mg./hr. |
|-------------|-----------------------------------------------------------------------------------------|-------------------------------------------------------------------------|-------------------------------------------------------------|----------------------------------------------------------------|------------------------------------------------------|-------------------------------------------|-----------------------------|---------------------------|
| XVI         | Allyl stearate-maleic anhydride, 1/1 copolymer.                                         | Lauryl methacrylate-maleic anhydride, 20/1 copolymer.                   | Polyethylene glycol, 550 mole weight monomethyl ether.      | Octadecyl amide.                                               | 35/52/7/6                                            | 2.5                                       | 7.5                         | 3.1                       |
| XVII        | do                                                                                      | do                                                                      | do                                                          | Octadecyl ammonium                                             | 35/52/7/6                                            | 2.5                                       | 7.8                         | 3.8                       |
| XVIII       | do                                                                                      | Lauryl methacrylate-maleic anhydride, 10/1 copolymer.                   | Polyethylene glycol, 550 mole weight mono-laurel ether.     | Hydroxyethyl amido.                                            | 33/50/12/5                                           | 2.5                                       | 8.0                         | 2.9                       |
| XIX         | do                                                                                      | Lauryl methacrylate-maleic anhydride, 30/1 copolymer.                   | do                                                          | Tetraethylene pentammonium.                                    | 30/55/12/3                                           | 2.5                                       | 6.9                         | 3.9                       |
| XX          | do                                                                                      | Lauryl methacrylate-maleic anhydride, 20/1 copolymer.                   | Polyethylene glycol, 400 mole weight.                       | 2,2,2-trihydroxy methylpropanoxy (pentaerythritol ester).      | 34/58/5/3                                            | 2.5                                       | 8.4                         | 3.8                       |
| XXI         | do                                                                                      | Allyl stearate-maleic anhydride-lauryl methacrylate, 1/15 copolymer.    | Poly-1,2-propylene glycol, 350 mole weight.                 | 2-mercapto propanoxy                                           | 25/53/10/2                                           | 2.5                                       | 6.5                         | 3.9                       |
| XXII        | do                                                                                      | do                                                                      | Polyethylene glycol, 550 mole weight                        | Triethanol ammonium.                                           | 39/48/7/6                                            | 2.5                                       | 8.7                         | 3.0                       |
| XXIII       | Vinyl stearate-maleic anhydride, 1/1 copolymer.                                         | Allyl stearate-maleic anhydride-vinyl 2-ethylhexoate, 1/1/30 copolymer. | Poly-1,2-propylene glycol, 500 mole weight monoethyl ether. | 3-morpholine amido.                                            | 33/57/6/4                                            | 2.5                                       | 7.2                         | 3.3                       |
| XXIV        | do                                                                                      | do                                                                      | do                                                          | 2,2-hydroxymethyl 3-oleoxy, propanoxy-N-(2-amino ethyl) amido. | 33/57/6/4                                            | 2.5                                       | 8.5                         | 3.1                       |
| XXV         | do                                                                                      | Vinyl stearate-maleic anhydride-cetyl acrylate, 1/1/18 copolymer.       | Polyethylene glycol, 550 mole weight monomethyl ether.      | do                                                             | 25/61/11/3                                           | 2.5                                       | 9.0                         | 3.1                       |
| XXVI        | Allyl stearate-maleic anhydride-maleamic acid, 1/0.9/0.1.                               | Lauryl methacrylate-maleic anhydride, 20/1 copolymer.                   | Polyethylene glycol, 400 mole weight.                       | Amido—see (A) component.                                       | 37/55/8                                              | 2.5                                       | 8.5                         | 3.0                       |
| XXVII       | Allyl stearate-maleic anhydride-maleimide, 1/0.9/0.1.                                   | Allyl stearate-maleic anhydride-lauryl acrylate, 1/1/30 copolymer.      | Polyethylene glycol, 750 mole weight monolauryl ether.      | Imide and amido—see (A) component.                             | 40/54/6                                              | 2.5                                       | 9.1                         | 2.9                       |
| XXVIII      | Methallyl stearate-maleic anhydride-isobutyl maleamide, 1/0.8/0.2 copolymer.            | Methallyl stearate-maleic anhydride-lauryl acrylate, 1/1/30 copolymer.  | do                                                          | Isobutyl amido—see (A) component.                              | 36/52/12                                             | 2.5                                       | 9.2                         | 2.9                       |
| XXIX        | Methallyl stearate-maleic anhydride-ethylene glycol monomaleate, 1/0.85/0.15 copolymer. | do                                                                      | do                                                          | 2-hydroxy ethoxy—see (A) component.                            | 27/63/10                                             | 1.5                                       | 9.0                         | 3.1                       |
| XXX         | Vinyl 2-ethyl-hexoate-maleic anhydride-octyl maleamate, 1/0.95/0.05 copolymer.          | Allyl stearate-maleic anhydride-lauryl methacrylate, 1/1/30 copolymer.  | Polyethylene glycol, 550 mole weight monomethyl ether.      | Amido—see (A) component.                                       | 40/56/4                                              | 2.5                                       | 8.7                         | 3.3                       |
| XXXI        | Allyl stearate-maleic anhydride-maleic acid, 1/0.5/0.2 copolymer.                       | Lauryl methacrylate-diisobutylene maleic anhydride, 18/10/1 copolymer.  | Polyethylene glycol, 400 mole weight.                       | Free acid—see (A) component.                                   | 34/51/15                                             | 2.5                                       | 8.9                         | 3.7                       |

TABLE II—Continued

| Example No. | (A) Component                                   | (B) Component                                                                           | Polyalkylene glycol                                    | Maleic anhydride polar substituent group (C) | Proportions of (A), (B) poly-alkylene glycol | Percent by weight additive in composition | Average piston varnish rate | Piston ring wear, mg./hr. |
|-------------|-------------------------------------------------|-----------------------------------------------------------------------------------------|--------------------------------------------------------|----------------------------------------------|----------------------------------------------|-------------------------------------------|-----------------------------|---------------------------|
| XXXII       | Allyl stearate-maleic anhydride, 1/1 copolymer. | Vinyl trimethyl-nonyl ether-dilauryl maleate maleic anhydride, 10/9/1 copolymer.        | Polyethylene glycol, 400 mole weight monolauryl ether. | 2-ethylhexyl amido.....                      | 42/45/8/5                                    | 2.5                                       | 7.5                         | 3.6                       |
| XXXIII      | do                                              | Cetyl phenoxyethyl methacrylate - maleic anhydride, 20/1 copolymer.                     | Polyethylene glycol, 800 mole weight monoctyl ether.   | Octyl thio.....                              | 40/42/10/8                                   | 2.5                                       | 8.4                         | 3.9                       |
| XXXIV       | do                                              | Vinyl stearyl ketone-maleic anhydride, 15/1 copolymer.                                  | Polyethylene glycol, 400 mole weight.                  | Dihydroxyethyl ethylene diammonium.          | 15/70/11/4                                   | 2.5                                       | 7.9                         | 4.0                       |
| XXXV        | do                                              | Vinyl stearyl ketone-dinonyl phenoxyethyl acrylate-maleic anhydride, 10/12/1 copolymer. | Polyethylene glycol, 550 mole weight monomethyl ether. | 2-nitro ethoxy.....                          | 15/70/9/6                                    | 2.5                                       | 7.2                         | 3.8                       |

In the above illustrated copolymers, the (C) component is present in a weight ratio of up to 2 parts of (C) for each part of the (B) copolymer; preferably, as illustrated by the above test data, the proportion of the (C) component will vary from about 0.05 to 1.0 for each part of the (B) component.

The compositions of the invention may also include other agents such as oiliness agents, viscosity index improvers, pour point depressants, blooming agents, peptizing agents, etc., as are known to the art. Although the compositions have been primarily described as crankcase lubricants for internal combustion engines, they are also useful as turbine oils, hydraulic fluids, instrument oils, oils for grease manufacture, ice machine oils and the like.

This application is a continuation-in-part of Stewart, Wilgus, and Stuart application Serial No. 549,871, filed November 29, 1955, and now abandoned, which in turn is a continuation-in-part of Stewart, Wilgus, and Stuart application Serial No. 479,224, filed December 31, 1954 (now abandoned), and of Stuart, Stewart, and Wilgus application Serial No. 549,870, filed November 29, 1955 and now abandoned, which in turn is a continuation-in-part of Stuart, Stewart, and Wilgus application Serial No. 479,239, filed December 31, 1954 (now abandoned).

We claim:

1. A lubricant composition comprising a major portion of an oil of lubricating viscosity and a minor portion, sufficient to enhance the detergent characteristics of the composition, of an oil-soluble mixture of (A) the copolymer of a monomer selected from the group consisting of (1) a fatty acid ester of an unsaturated alcohol, said fatty acid containing 8 to 30 carbon atoms and said unsaturated alcohol being selected from the group consisting of  $\alpha$  and  $\beta$ -unsaturated alcohols containing up to 7 carbon atoms, (2) 1-olefins of 6 to 24 carbon atoms and (3) vinyl and allyl alkyl ethers having 4 to 22 carbon atoms in the alkyl group with maleic anhydride, said monomers being in approximately 1:1 molar ratio, and (B) the copolymer of monomers selected from at least the first two classes of the groups consisting of (1) maleic anhydride (2) a higher alkyl ester of an  $\alpha$ , $\beta$ -unsaturated monocarboxylic acid of from 3 to 8 carbon atoms of which the alkyl group contains from 8 to 30 carbon atoms and (3) a fatty acid ester of an unsaturated alcohol in which the fatty acid contains up to 30 carbon atoms and the unsaturated alcohol is a member of the group consisting of  $\alpha$  and  $\beta$ -unsaturated alcohols containing up to 20 carbon atoms, at least one of said (A) and (B) copolymers being partially esterified with a member of the group consisting of polyalkylene glycols having a molecular weight between about 106 and 10,000 and alkyl ethers thereof in which the alkylene groups contain from 2 to 7 carbon atoms each and the alkyl groups contain from 1 to 30 carbon atoms each and said (A) and (B) copolymers being in the weight ratio of 0.15 to 5 parts of (A) for each part of (B).

2. A lubricant composition comprising a major portion of an oil of lubricating viscosity and from about 0.1 to 10% by weight of an oil-soluble mixture of (A) the copolymer of an allyl ester of a fatty acid, said fatty acid containing 8 to 30 carbon atoms, with maleic anhydride in approximately 1:1 molar ratio and (B) the copolymer of maleic anhydride and a higher alkyl ester of  $\alpha$ , $\beta$ -unsaturated monocarboxylic acid of from 3 to 8 carbon atoms, in which the alkyl group contains from 8 to 30 carbon atoms the total maleic anhydride of said (A) and said (B) copolymers being 2 to 75% esterified with a polyethylene glycol having a molecular weight between about 200 and about 2000 and said (A) and (B) copolymers being in the weight ratio of 0.15 to 5 parts of (A) for each part of (B).

3. A lubricant composition comprising a major portion of an oil of lubricating viscosity and from about 0.1 to 10%, by weight, of an oil-soluble mixture of the copolymer of allyl stearate with maleic anhydride in approximately 1:1 molar ratio and the copolymer of maleic anhydride and lauryl methacrylate, the total maleic anhydride of said mixture of copolymers being 2-75% esterified with a polyethylene glycol monoalkyl ether having a molecular weight between about 200 and 2,000, and from 1 to 30 carbon atoms in the alkyl group, and said copolymers being in the weight ratio of 0.15 to 5 parts of the allyl stearate and maleic anhydride copolymer for each part of the maleic anhydride and lauryl methacrylate copolymer.

4. A lubricant composition comprising a major portion of an oil of lubricating viscosity and a minor portion, sufficient to enhance the detergent characteristics of the composition, of an oil-soluble mixture of (A) the copolymer of a monomer selected from the group consisting of (1) a fatty acid ester of an unsaturated alcohol, said fatty acid containing 8 to 20 carbon atoms and said unsaturated alcohol being selected from the group consisting of  $\alpha$  and  $\beta$ -unsaturated alcohols containing up to 7 carbon atoms, (2) 1-olefins of 6 to 24 carbon atoms and (3) vinyl and allyl alkyl ethers having 4 to 22 carbon atoms in the alkyl group with maleic anhydride, said monomers being in approximately 1:1 molar ratio, and (B) the copolymer of monomers selected from each of the groups consisting of (1) maleic anhydride (2) a higher alkyl ester of an  $\alpha$ , $\beta$ -unsaturated monocarboxylic acid of from 3 to 8 carbon atoms of which the alkyl group contains from 8 to 30 carbon atoms and (3) a fatty acid ester of an unsaturated alcohol in which the fatty acid contains up to 30 carbon atoms and the unsaturated alcohol is a member

5. A lubricant composition comprising a major portion of an oil of lubricating viscosity and a minor portion, sufficient to enhance the detergent characteristics of the composition, of an oil-soluble mixture of (A) the copolymer of a monomer selected from the group consisting of (1) a fatty acid ester of an unsaturated alcohol, said fatty acid containing 8 to 20 carbon atoms and said unsaturated alcohol being selected from the group consisting of  $\alpha$  and  $\beta$ -unsaturated alcohols containing up to 7 carbon atoms, (2) 1-olefins of 6 to 24 carbon atoms and (3) vinyl and allyl alkyl ethers having 4 to 22 carbon atoms in the alkyl group with maleic anhydride, said monomers being in approximately 1:1 molar ratio, and (B) the copolymer of monomers selected from each of the groups consisting of (1) maleic anhydride (2) a higher alkyl ester of an  $\alpha$ , $\beta$ -unsaturated monocarboxylic acid of from 3 to 8 carbon atoms of which the alkyl group contains from 8 to 30 carbon atoms and (3) a fatty acid ester of an unsaturated alcohol in which the fatty acid contains up to 30 carbon atoms and the unsaturated alcohol is a member

of the group consisting of  $\alpha$  and  $\beta$ -unsaturated alcohols containing up to 20 carbon atoms, at least one of said (A) and (B) copolymers being partially esterified with a member of the group consisting of polyalkylene glycols having a molecular weight between about 106 and 10,000 and alkyl ethers thereof in which the alkylene groups contain from 2 to 7 carbon atoms each and the alkyl groups contain from 1 to 30 carbon atoms each and said (A) and (B) copolymers being in the weight ratio of 0.15 to 5 parts of (A) for each part of (B).

5. A lubricant composition comprising a major portion of an oil of lubricating viscosity and from about 0.1 to 10% by weight of an oil-soluble mixture of (A) the copolymer of a fatty acid ester of unsaturated alcohol, said fatty acid containing 8 to 30 carbon atoms and said unsaturated alcohol being selected from the group consisting of  $\alpha$  and  $\beta$ -unsaturated alcohols containing up to 7 carbon atoms with maleic anhydride and (B) the copolymer of (1) maleic anhydride, (2) a higher alkyl ester of an  $\alpha,\beta$ -unsaturated monocarboxylic acid of from 3 to 8 carbon atoms of which the alkyl group contains from 8 to 30 carbon atoms and (3) a fatty acid ester of an unsaturated alcohol in which the fatty acid contains 8 to 30 carbon atoms and the unsaturated alcohol is a member of the group consisting of  $\alpha$  and  $\beta$ -unsaturated alcohols containing up to 7 carbon atoms, at least one of said (A) and (B) copolymers being partially esterified with a polyalkylene glycol having a molecular weight between 106 and about 10,000 in which the alkylene groups contain from 2 to 7 carbon atoms each and said (A) and (B) copolymers being in the weight ratio of 0.15 to 5 parts of (A) for each part of (B).

6. A lubricant composition comprising a major portion of an oil of lubricating viscosity and from about 0.1 to 10% by weight of an oil-soluble mixture of (A) the copolymer of an allyl ester of a higher fatty acid of from 8 to 30 carbon atoms with maleic anhydride and (B) the copolymer of (1) maleic anhydride, (2) a higher alkyl ester of an  $\alpha,\beta$ -unsaturated monocarboxylic acid of from 3 to 8 carbon atoms of which the alkyl group contains from 8 to 30 carbon atoms and (3) an allyl ester of a higher fatty acid of from 8 to 30 carbon atoms, at least one of said (A) and (B) copolymers being partially esterified with a polyethylene glycol having a molecular weight between about 200 and about 2,000 and said (A) and (B) copolymers being in the weight ratio of 0.15 to 5 parts of (A) for each part of (B).

7. A lubricant composition comprising a major portion of an oil of lubricating viscosity and from about 0.1 to 10% by weight of an oil-soluble mixture of (A) the copolymer of an allyl ester of a higher fatty acid of from 8 to 30 carbon atoms with maleic anhydride and (B) the copolymer of (1) maleic anhydride, (2) a higher alkyl ester of an  $\alpha,\beta$ -unsaturated monocarboxylic acid of from 3 to 8 carbon atoms in which the alkyl group contains from 8 to 30 carbon atoms and (3) an allyl ester of a higher fatty acid of from 8 to 30 carbon atoms, at least one of said (A) and said (B) copolymers being partially esterified with a polyethylene glycol monoalkyl ether having from 1 to 30 carbon atoms in the alkyl group and a molecular weight between about 200 and about 2,000 and said (A) and (B) copolymers being in the weight ratio of 0.15 to 5 parts of (A) for each part of (B).

8. A lubricant composition comprising a major portion of an oil of lubricating viscosity and from about 0.1 to 10% by weight of an oil-soluble mixture of (A) the copolymer of an allyl ester of a higher fatty acid of from 8 to 30 carbon atoms with maleic anhydride in approximately 1:1 molar ratio and (B) the copolymer of (1) maleic anhydride, (2) a higher alkyl ester of an  $\alpha,\beta$ -unsaturated monocarboxylic acid of from 3 to 8 carbon atoms in which the alkyl group contains from 8 to 30 carbon atoms and (3) an allyl ester of a higher fatty acid of from 8 to 30 carbon atoms, said copolymer containing

from about 0.25 to 4 moles of allyl ester for each mole of maleic anhydride, and the molar ratio of the higher alkyl ester being from about 5 to 50 times that of the combined maleic anhydride and allyl ester, said (A) and said (B) copolymers being present in approximately equal parts and partially esterified with a polyethylene glycol having a molecular weight between about 200 and about 2,000, the total molecular weight of the copolymer being at least 2,000.

9. A lubricant composition comprising a major portion of an oil of lubricating viscosity and from about 0.1 to 10% by weight of an oil-soluble mixture of (A) the copolymer of allyl stearate with maleic anhydride in approximately 1:1 molar ratio and (B) the copolymer of (1) maleic anhydride, (2) lauryl methacrylate and (3) allyl stearate, said copolymer containing about 0.25 to 4 moles of allyl stearate for each mole of maleic anhydride, and the lauryl methacrylate being present in molar proportions of 5 to 50 times that of the combined maleic anhydride and allyl stearate, said (A) and said (B) components being partially esterified with a polyethylene glycol monoalkyl ether having from 1 to 30 carbon atoms in the alkyl group and a molecular weight between 200 and about 2,000, from about 0.04 to 1.5 mole of polyethylene glycol being present for each mole of maleic anhydride in component (A) and the total molecular weight of the copolymer mixture being at least 2,000.

10. A lubricant composition comprising a major portion of an oil of lubricating viscosity and from about 0.1 to 10% by weight of an oil-soluble mixture of (A) the copolymer of vinyl stearate with maleic anhydride in approximately 1:1 molar ratio and (B) the copolymer of (1) maleic anhydride, (2) lauryl methacrylate and (3) allyl stearate, said copolymer containing about 0.25 to 4 moles of allyl stearate for each mole of maleic anhydride, and the lauryl methacrylate being present in the molar proportions of 5 to 50 times that of the combined maleic anhydride and allyl stearate, said (A) and said (B) components being partially esterified with a polyethylene glycol monoalkyl ether having from 1 to 30 carbon atoms in the alkyl group and a molecular weight between 200 and about 2,000, from about 0.04 to 1.5 moles of polyethylene glycol being present for each mole of maleic anhydride in component (A) and the total molecular weight of the copolymer mixture being at least 2,000.

11. A lubricant composition comprising a major portion of an oil of lubricating viscosity and from about 0.1 to 10% by weight of an oil-soluble mixture of (A) the copolymer of octadecene-1 with maleic anhydride in approximately 1:1 molar ratio and (B) the copolymer of (1) maleic anhydride, (2) lauryl methacrylate and (3) allyl stearate, said copolymer containing about 0.25 to 4 moles of allyl stearate for each mole of maleic anhydride, and the lauryl methacrylate being present in the molar proportions of 5 to 50 times that of the combined maleic anhydride and allyl stearate, said (A) and said (B) components being partially esterified with a polyethylene glycol monoalkyl ether having from 1 to 30 carbon atoms in the alkyl group and a molecular weight between 200 and about 2,000, from about 0.04 to 1.5 moles of polyethylene glycol being present for each mole of maleic anhydride in component (A) and the total molecular weight of the copolymer mixture being at least 2,000.

12. A lubricant composition comprising a major portion of an oil of lubricating viscosity and from about 0.1 to 10% by weight of an oil-soluble mixture of (A) the copolymer of vinyl 2-ethyl hexyl ether with maleic anhydride in approximately 1:1 molar ratio and (B) the copolymer of (1) maleic anhydride, (2) lauryl methacrylate and (3) allyl stearate, said copolymer containing about 0.25 to 4 moles of allyl stearate for each mole of maleic anhydride, and the lauryl methacrylate being present in molar proportions of 5 to 50 times that of the combined maleic anhydride and allyl stearate, said (A)

and said (B) components being partially esterified with a polyethylene glycol monoalkyl ether having from 1 to 30 carbon atoms in the alkyl group and a molecular weight between 200 and about 2,000, from about 0.04 to 1.5 moles of polyethylene glycol being present for each mole of maleic anhydride in component (A) and the total molecular weight of the copolymer mixture being at least 2,000.

13. A lubricant composition comprising a major portion of an oil of lubricating viscosity and from about 0.1 to 10% by weight of an oil-soluble mixture of (A) the copolymer of allyl stearate and vinyl 2-ethylhexyl ether with maleic anhydride in approximately 0.25:0.75:1 molar ratio and (B) the copolymer of (1) maleic anhydride, (2) lauryl methacrylate and (3) allyl stearate, said copolymer containing about 0.25 to 4 moles of allyl stearate for each mole of maleic anhydride, and the lauryl methacrylate being present in molar proportions of 5 to 50 times that of the combined maleic anhydride and allyl stearate, said (A) and said (B) components

5

15

20

being partially esterified with a polyethylene glycol monoalkyl ether having from 1 to 30 carbon atoms in the alkyl group and a molecular weight between 200 and about 2,000, from about 0.04 to 1.5 moles of polyethylene glycol being present for each mole of maleic anhydride in component (A) and the total molecular weight of the copolymer mixture being at least 2,000.

## References Cited in the file of this patent

## UNITED STATES PATENTS

|           |                   |               |
|-----------|-------------------|---------------|
| 2,615,844 | Giannmaria        | Oct. 28, 1952 |
| 2,615,845 | Lippincott et al. | Oct. 28, 1952 |
| 2,684,355 | Van Horne         | July 20, 1954 |
| 2,694,685 | Bartlett          | Nov. 16, 1954 |
| 2,704,277 | Giannmaria        | Mar. 15, 1955 |
| 2,731,448 | Bauer et al.      | Jan. 17, 1956 |
| 2,737,496 | Catlin            | Mar. 6, 1956  |

## FOREIGN PATENTS

|               |               |
|---------------|---------------|
| Great Britain | Feb. 20, 1957 |
|---------------|---------------|

768,701